

## UNITED STATES PATENT OFFICE

2,224,245

## PROTECTION OF MAGNESIUM-RICH ALLOYS

Frank Arthur Allen, Windsor, England, assignor  
to High Duty Alloys Limited, Slough, EnglandNo Drawing. Application February 7, 1939, Se-  
rial No. 255,165. In Great Britain September  
13, 1938

9 Claims. (Cl. 148—6)

This invention relates to the protection against corrosion and erosion of articles composed of or including portions composed of magnesium rich alloys.

5 The employment of magnesium rich alloys has heretofore been considerably restricted owing to their low resistance to corrosion by sea water and other causes and to erosion, the resistance varying inversely with the magnesium content 10 and being least in magnesium base alloys in which magnesium predominates, and the present invention has for its object to remove this disadvantage.

In accordance with the present invention, the 15 process for the treatment of articles composed of, or including portions composed of, magnesium rich alloys consists in immersing the article or the relevant portion thereof in a heated aqueous solution of alkali dichromate and nickel sulphate, chromium sulphate or nickel ammonium sulphate 20 to which has been added an organic acidifying agent producing in such aqueous solution or maintaining it at a pH value between 2.0 and 6.4 and which value is advantageously not less than 25 3.4 and not greater than 4.4.

The acidification of the aqueous solution considerably facilitates the process and improves the protective deposit and the organic acidifying agents employed according to the present invention 30 are preferably those which only slightly ionise in solution and therefore successively liberate further hydrogen ions as the process continues thus maintaining the concentration in chemical equilibrium, examples of such agents being organic acids and salts thereof.

Preferably also the pH value of the aqueous solution is adjusted to 3.8 as is that of the organic acidifying addition which may conveniently be made up of acetic acid and sodium or ammonium acetate.

40 In the practice of the invention according to one mode of carrying out the process, 50 gallons of solution is made up of the following composition:

|                           |       |       |
|---------------------------|-------|-------|
| 45 1.5% Chromium sulphate | lbs.  | 7 1/2 |
| 3.0% Potassium dichromate | lbs.  | 15    |
| 0.625% Acetic acid        | pints | 2 1/2 |
| 0.8% Sodium acetate       | lbs.  | 4     |
| Water to make 50 gallons. |       |       |

50 Die castings acid dipped in 5% sulphuric acid and immersed in this solution at boiling point chromate perfectly, without difficulty, in 20 minutes, there being no necessity for any acid addition and the reaction being gentle with the

semblance that the deposit darkens from dark brown to black on drying. The treated castings have a clean, smooth, shiny surface.

Other combinations of organic acids and salts giving the same pH range could be used to maintain the equilibrium of the solution and further other concentrations of chromium sulphate, and potassium dichromate giving a pH value of less than 4.4 could be used so long as acidified solutions of the same pH as the resultant aqueous 10 solution are also employed.

Another aspect of the present invention consists in the preliminary treatment of stampings, sand castings or dirty articles including or composed of magnesium rich alloys with a view to 15 ensuring a satisfactory deposit on immersion.

This pretreatment is effected in a bath, preferably cold, consisting of 5-20% chromic acid and 2-10% nitric acid in water, which is found effectively to remove partly carbonized grease and embedded dirt in stampings and the like in ten minutes and when followed by a quick sulphuric acid dip, gives perfectly bright articles. The preferred composition is 8% chromic acid and 5% nitric acid. It is noteworthy that the action of this 25 chromic/nitric acid bath is quite gentle and much less vigorous than that of either of the component acids separately.

By the present invention improved processes for the protection of articles composed of, or including portions composed of, magnesium rich 30 alloys are obtained.

What I claim is:

1. A process for the treatment of articles composed of magnesium rich alloys consisting in immersing the article in an aqueous solution of alkali dichromate and metallic sulphate to which has been added an organic acidifying agent maintaining such aqueous solution at a pH value between 2.0 and 6.4. 35

2. A process for the treatment of articles composed of magnesium rich alloys consisting in immersing the article in a heated aqueous solution of alkali dichromate and metallic sulphate to which aqueous solution has been added an organic acidifying agent rendering and maintaining it at a pH value between 3.4 and 4.3. 45

3. A process according to claim 2, wherein the acidifying agents consist of organic acids and salts which only slightly ionise in solution and therefore successively liberate further ions as the process continues. 50

4. A process for the treatment of articles composed of magnesium rich alloys consisting in immersing the article in a heated aqueous solution 55

of alkali dichromate and metallic sulphate, to which has been added an organic acidifying agent, the pH value of such aqueous solution and of the organic addition being each adjusted to 3.8.

5. A process according to claim 2 wherein the acidifying addition consists of acetic acid and sodium acetate.

6. A process according to claim 2 wherein the organic acidifying addition consists of acetic acid and ammonium acetate.

10. 7. A process according to claim 2 wherein the aqueous solution contains the following ingredients per 50 gallons:

|    |                           |       |    |
|----|---------------------------|-------|----|
| 15 | 1.5% Chromium sulphate    | lbs   | 7½ |
|    | 3.0% Potassium dichromate | lbs   | 15 |
|    | 0.625% Acetic acid        | pints | 2½ |
|    | 0.8% Sodium acetate       | lbs   | 4  |

8. A process according to claim 2 when applied to stampings, sand castings and dirty articles including the preliminary step of immersing the articles in a bath consisting of 8% chromic acid and 5% nitric acid in water, whereby grease and embedded dirt is removed.

9. A process according to claim 2 when applied to stampings, sand castings and dirty articles including the preliminary step of immersing the articles in a bath consisting of 8% chromic acid 10 and 5% nitric acid in water, whereby grease and embedded dirt is removed, such pretreatment including a quick sulphuric acid dip.

FRANK ARTHUR ALLEN. 15